

3,261,674  
**STABILIZED GASOLINE ANTIKNOCK COMPOSITIONS AND GASOLINE CONTAINING SAME**  
Albert C. Condo, Jr., Newtown Square, Pa., assignor to  
The Atlantic Refining Company, Philadelphia, Pa., a  
corporation of Pennsylvania  
No Drawing. Filed Mar. 10, 1961, Ser. No. 94,686  
12 Claims. (Cl. 44—69)

This invention relates to improved fuel for spark ignition internal combustion engines and to additive compositions for such fuel. More particularly, this invention relates to gasoline compositions containing a cyclopentadienyl manganese tricarbonyl antiknock agent and a beta-diketone.

Recently there has been developed a new class of organometallic antiknock agents for gasoline fuels employed in spark ignition internal combustion engines. These agents are the cyclopentadienyl manganese tricarbonyls. The synthesis of the cyclopentadienyl manganese tricarbonyls, the use of such compounds as antiknock agents for gasoline fuels, and other gasoline additives that can be associated therewith are set forth in U.S. Patents No. 2,818,416, No. 2,818,417, and No. 2,870,180. A considerable amount of antiknock data have been obtained on the methyl cyclopentadienyl manganese tricarbonyl compound the synthesis of which is described in Example II of the aforementioned Patent No. 2,870,180. These antiknock data are reported in the article by J. E. Brown and W. G. Lovell, entitled "A New Manganese Antiknock," in Industrial and Engineering Chemistry, volume 50, page 1547, et seq. (1958). These data show that, in particular, methyl cyclopentadienyl manganese tricarbonyl may be utilized as the sole antiknock agent in commercial motor gasolines and also that such manganese antiknock agents can be used in combination with lead alkyl antiknock agents, in particular tetraethyl lead. Moreover, it was found that the manganese antiknock compound exhibited a particularly marked synergistic effect on the antiknock characteristics of the gasoline when small amounts, i.e. from 0.1 to 0.5 gram of manganese in the form of the methyl cyclopentadienyl manganese tricarbonyl per gallon of gasoline, are used in conjunction with 2 or 3 milliliters of tetraethyl lead per gallon of gasoline.

It has been found, however, that although the cyclopentadienyl manganese tricarbonyls will not decompose and will remain in solution in gasoline as long as they or the gasoline containing them is not exposed to radiation such as sunlight, they are unstable in the presence of radiation such as sunlight and will decompose or will precipitate out of the gasoline in the form of a dark-colored precipitate, generally a dark brown precipitate. Moreover, if the manganese compound is utilized in a gasoline containing a lead antiknock agent such as tetraethyl lead, this instability also causes a white precipitate of lead to form on top of the dark brown precipitate. This is particularly surprising since tetraethyl lead is stable in gasoline in the presence of sunlight over relatively long periods of time when there is no cyclopentadienyl manganese tricarbonyl compound present in the gasoline.

It has now been found that the cyclopentadienyl manganese tricarbonyls can be inhibited against a precipitate-forming decomposition reaction resulting from exposure to sunlight by incorporating a beta diketone in the cyclopentadienyl manganese tricarbonyl and the cyclopentadienyl manganese tricarbonyls can be retained in solution in gasoline in the presence of sunlight if a beta-diketone is also contained in the gasoline.

It is an object of this invention, therefore, to provide a stable antiknock additive for spark ignition internal combustion engine fuels.

It is another object of this invention to provide a stable antiknock additive containing a cyclopentadienyl manganese tricarbonyl antiknock agent and a beta diketone for spark ignition internal combustion engine fuels.

It is another object of this invention to provide a stable antiknock additive containing a lead alkyl antiknock agent, a cyclopentadienyl manganese tricarbonyl antiknock agent, and a beta-diketone for spark ignition internal combustion engine fuels.

It is another object of this invention to provide a fuel composition for use in spark ignition internal combustion engines containing a cyclopentadienyl manganese tricarbonyl antiknock agent and a beta-diketone.

It is another object of this invention to provide a fuel composition for use in spark ignition internal combustion engines containing a lead alkyl antiknock agent, a cyclopentadienyl manganese tricarbonyl antiknock agent, and a beta diketone.

Other objects of this invention will be apparent from the detail description of the invention and the claims that follow.

In accordance with this invention from 1 to 3 moles of a hydrocarbon oil soluble beta diketone will inhibit one mole of a cyclopentadienyl manganese tricarbonyl antiknock agent against a precipitate-forming decomposition reaction resulting from exposure to radiation such as sunlight. Further, in accordance with another embodiment of this invention, from 1 to 3 moles of a hydrocarbon oil soluble beta diketone per mole of cyclopentadienyl manganese tricarbonyl antiknock agent when added to a stable gasoline containing the cyclopentadienyl manganese tricarbonyl antiknock agent will prevent the manganese compound from precipitating out of solution when such gasoline is exposed to radiation such as sunlight. The hydrocarbon oil soluble beta diketones of this invention are characterized by having the structural formula



wherein R and R' are hydrocarbon radicals selected from the group consisting of alkyl, aryl, alkaryl and aralkyl radicals containing from 1 to 20 carbon atoms and wherein R and R' may be the same or different. As used herein, the term "hydrocarbon oil" includes gasoline boiling range hydrocarbon fractions, light naphtha fractions and the like. The gasoline may also contain other additives, in particular, a lead alkyl antiknock agent such as tetraethyl lead, in addition to the cyclopentadienyl manganese tricarbonyl compound, without affecting the stabilizing properties of the beta-diketone or the manganese compound.

The stable gasoline fuel to which the antiknock compositions of this invention are added is a petroleum fraction boiling in the gasoline hydrocarbon range, i.e. between about 50° F. and about 450° F., and which gasoline fuel is relatively stable with respect to oxidation or gum formation. The stability may result from the use of stable base stocks such as alkylate, reformate and the like

which have been highly refined to remove olefins, or the stability may result from the use of conventional oxidation inhibitors. In addition, such fuels may contain conventional anti-rust additives, carburetor anti-icing additives, pre-ignition inhibitors such as the phosphorus compounds, dyes, and similar compounds which are conventionally added to gasoline.

The gasoline may also contain from 0.1 gram to 6.3 grams of lead per gallon, the lead being in the form of an

organolead, antiknock agent such as lead alkyl, for example, tetraethyl lead, tetra-methyl lead, tetra-methyl-ethyl lead, tetra-isopropyl lead and the like. In addition to the lead compound, the lead antiknock agent contains the usual scavenging agents such as ethylene dibromide and ethylene dichloride.

The cyclopentadienyl manganese tricarbonyl antiknock agent such as the cyclopentadienyl manganese tricarbonyl or the alkyl cyclopentadienyl manganese tricarbonyl, for example, the methyl cyclopentadienyl compound, is added to the gasoline in amounts such that the manganese of the cyclopentadienyl manganese tricarbonyl compound ranges from 0.1 gram to 6.3 grams per gallon of the gasoline. The amount of oil soluble beta diketone required to be added together with the manganese compound ranges between 1 mole and 3 moles per mole of the cyclopentadienyl manganese tricarbonyl.

In another embodiment of the invention the cyclopentadienyl manganese tricarbonyl antiknock agent is combined with the lead alkyl antiknock fluid to give a combination antiknock agent for addition to gasoline. In these compositions the weight ratio of the manganese of the cyclopentadienyl manganese tricarbonyl compound to the lead of the lead alkyl ranges from 1:63 to 1:1 and preferably from 1:24 to 1:2 in order to obtain the desired octane appreciation. In these compositions the mole ratio of the beta diketone inhibitor to the manganese compound ranges from 1:1 to 3:1 in order to prevent the manganese compound from decomposing and precipitating out of solution when such composition is exposed to sunlight.

A test was developed in order to demonstrate the effectiveness of the oil soluble beta diketones of this invention as compared with other diketones and similar compounds for inhibiting the radiation induced decomposition of the cyclopentadienyl manganese tricarbonyls.

A premium type grade gasoline comprising hydrocarbons in the boiling range between 90° F. and 400° F. obtained by blending products predominantly from catalytic cracking, catalytic reforming and alkylation and containing 3 cc. of tetraethyl lead per gallon to give a fuel having an octane number of 100 by the ASTM Method D908 was selected as the gasoline component for the various compositions to be compared. The desired quantity of methyl cyclopentadienyl manganese tricarbonyl was added to the gasoline component. In Examples I and II this amount corresponded to 0.5 gram of manganese per gallon of gasoline. The desired amount of each compound to be tested for inhibition was then added to the gasoline containing the manganese compound. In Examples I and II this amount corresponded to 3 moles per mole of the methyl cyclopentadienyl manganese tricarbonyl for the individual compositions to be compared. In Examples I, II, III, and IV the individual compositions were placed in stoppered, clear glass bottles and exposed to diffuse daylight in the laboratory. In Examples I and II they were observed each day and the time when the first precipitate appeared was noted. The leaded gasoline component without the addition of any cyclopentadienyl manganese tricarbonyl compound or beta diketone remained completely clear upon exposure to the laboratory daylight and no precipitate formed.

## EXAMPLE I

In order to demonstrate the criticality of the beta diketones as the class of compounds which inhibit radiation induced precipitate-forming decomposition reactions of the cyclopentadienyl manganese tricarbonyls, the comparisons shown in Table I were made on gasoline solutions prepared as has been described.

|    |                                      | Table I | Days until ppt. appeared |
|----|--------------------------------------|---------|--------------------------|
| 10 | Inhibitor compound tested:           |         |                          |
|    | Blank—no inhibitor                   | -----   | 8                        |
|    | 2,3-butanedione (an alpha-diketone)  | -----   | 8                        |
|    | 2,5-hexanedione (a gamma-diketone)   | -----   | 8                        |
|    | 2,4-pentanedione (a beta-diketone)   | -----   | 10-11                    |
|    | Isovaleryl acetone (a beta-diketone) | -----   | <sup>1</sup> >21         |
|    | Diethyl malonate                     | -----   | 8                        |
|    | Ethyl acetoacetate                   | -----   | 8                        |
| 15 | Dimethyl maleate                     | -----   | 10                       |
|    | Diethyl oxalate                      | -----   | 6                        |

<sup>1</sup> No precipitate observable after 21 days, test discontinued.

These data show that the beta diketones are superior to the other classes of diketones and to compounds having structures similar to the diketones.

## EXAMPLE II

A number of oil soluble beta-diketones representative of various types of groups attached to the diketone nucleus were tested in the same manner as described for Example I. The solutions were allowed to stand in daylight for 21 days and then they were filtered and the amount of precipitate per 100 cc. of solution was determined. The results are shown in Table II.

|    |                                 | Table II                 | Mg. of ppt., per 100 cc. of solution after 21 days |
|----|---------------------------------|--------------------------|----------------------------------------------------|
|    | Beta diketone tested            | Days until ppt. appeared |                                                    |
| 40 | Blank, no inhibitor             | -----                    | 70                                                 |
|    | 2,4-pentanedione                | 8                        | 17.5                                               |
|    | 2,4-decanedione                 | 11                       | 7                                                  |
|    | Isovaleryl acetone              | 21                       |                                                    |
| 45 | 5,5'-dimethylhexanedione        | 1 >21                    |                                                    |
|    | 4-phenyl-2,4-butanedione        | 16                       | 23                                                 |
|    | 4-methyl phenyl-2,4-butanedione | 16                       | 21                                                 |
|    | Diisovaleryl methane            | 16                       | 37                                                 |
|    |                                 | 10                       | 27                                                 |

<sup>1</sup> No ppt. after 21 days, test discontinued.

These data show that a wide variety of oil soluble beta diketones are excellent inhibitors for preventing the precipitation of decomposed cyclopentadienyl manganese tricarbonyls contained in gasoline exposed to daylight. They also show that not all of these compounds have the same inhibiting properties and that isovaleryl acetone is particularly preferred.

## EXAMPLE III

Several additive compositions were prepared and tested by allowing them to stand in stoppered, clear glass bottles exposed to laboratory daylight. They were observed after one day and again after seven days exposure. The compositions and results are set forth in Table III.

| Composition                                                                                                                                                                               | After one day          | After seven days         |
|-------------------------------------------------------------------------------------------------------------------------------------------------------------------------------------------|------------------------|--------------------------|
| Methyl cyclopentadienyl manganese tricarbonyl                                                                                                                                             | Some precipitate       | Heavy, dark precipitate. |
| 0.7 gram methyl cyclopentadienyl manganese tricarbonyl, 3 cc. tetraethyl lead motor mixture, Isovaleryl acetone in an amount corresponding to 3 moles per mole of the manganese compound. | Clear, no precipitate  | Clear, no precipitate.   |
| Methyl cyclopentadienyl manganese tricarbonyl, Isovaleryl acetone in an amount corresponding to 1 mole per mole of the manganese compound.                                                | Very slightly darkened | Dark, no precipitate.    |

These tests demonstrate that stable compositions for addition to gasoline may be prepared containing the cyclopentadienyl manganese tricarbonyl antiknock agent and the beta diketone.

#### EXAMPLE IV

The same gasoline base fuel containing 3 cc. of tetraethyl lead per gallon employed in Examples I and II was used to make up a series of solutions to show the effect of the inhibitors of this invention on octane number of the gasoline. The octane numbers were measured by ASTM Method D1656-60T. Methyl cyclopentadienyl manganese tricarbonyl at two different manganese levels were tested with and without isovaleryl acetone inhibitor under the conditions and with the results shown in Table IV.

Table IV

| Gms. Mn.,<br>Per Gal. | Mole ratio Iso-<br>valeryl Ace-<br>tone to Mn.<br>Compound | Days<br>Stored | Storage<br>Condition | Observation<br>at end of<br>Storage Period | Octane<br>Number<br>After<br>Storage |
|-----------------------|------------------------------------------------------------|----------------|----------------------|--------------------------------------------|--------------------------------------|
| 0.125                 |                                                            | 7              | Darkness             | Clear, no ppt.                             | 102.5                                |
| 0.125                 |                                                            | 7              | Daylight             | Dark brown ppt.                            | 100.4                                |
| 0.125                 | 3/1                                                        | 7              | do                   | Clear, no ppt.                             | 102.0                                |
| 0.50                  |                                                            | 10             | Darkness             | do                                         | 103.4                                |
| 0.50                  |                                                            | 10             | Daylight             | Dark brown ppt. <sup>1</sup>               | 101.9                                |
| 0.50                  | 3/1                                                        | 10             | do                   | Clear, no ppt.                             | 102.6                                |

<sup>1</sup> This precipitate analyzed, and found to contain 20.3 weight percent manganese, 3.0 weight percent lead, 23.0 weight percent carbon and 3.8 weight percent hydrogen.

These data show that no precipitate forming decomposition reactions occur if the gasoline containing the methyl cyclopentadienyl tricarbonyl with no inhibitor is stored in the dark. Moreover, the octane appreciation above the 100 octane number value for the leaded base gasoline remains normal for the quantities of methyl cyclopentadienyl tricarbonyl employed. The data also show that if the gasoline containing the methyl cyclopentadienyl tricarbonyl is exposed to daylight with no inhibitor, the manganese compound precipitates and the octane number appreciation due to synergistic effect of the manganese compound is greatly reduced. If, however, a hydrocarbon oil soluble beta diketone inhibitor is employed with the cyclopentadienyl manganese tricarbonyl compound the manganese compound does not precipitate in the presence of daylight and the octane number appreciation due to the synergistic action of the manganese compound is retained with only minor reductions.

#### EXAMPLE V

Several solutions were prepared in the same base gasoline as that employed in Examples I, II, and IV. These solutions were stored in stoppered, glass bottles, but instead of being exposed to ordinary diffuse daylight in the laboratory as in the previous examples, they were exposed to direct, intense sunlight. The compositions tested and the results observed are shown in Table V. The manganese compound was methyl cyclopentadienyl tricarbonyl and the inhibitor was isovaleryl acetone in all solutions where such compounds were employed.

Table V

| Gms. Mn.,<br>Per Gal. | Inhibitor | Mole ratio<br>Inhib. to<br>Mn. Compd. | Appearance                   |                                 |
|-----------------------|-----------|---------------------------------------|------------------------------|---------------------------------|
|                       |           |                                       | After 2 days Exposure        | After 8 days Exposure           |
| 0                     | No        |                                       | Clear, no ppt.               | Clear, no ppt.                  |
| 0                     | Yes       | (1)                                   | do                           | Do.                             |
| 0.5                   | No        |                                       | Large amount dark brown ppt. | Large amount dark brown ppt.    |
| 0.5                   | Yes       | 3:1                                   | Clear, no ppt.               | Clear, no ppt.                  |
| 0.5                   | Yes       | 1:1                                   | Sl. cloudy solution          | Small to medium amount of ppt.  |
| 0.5                   | Yes       | 1:2                                   | Small amount of ppt.         | Large amount of dark brown ppt. |

<sup>1</sup> 0.98 gm. per gal.

These data show that the base gasoline component was stable in the presence of direct, intense sunlight and that

this stability was not affected by the presence of the inhibitor compound. The data also show that it is necessary to employ at least a 1:1 mole ratio of the beta diketone inhibitor to the cyclopentadienyl manganese tricarbonyl compound to provide protection against the precipitate-forming decomposition reactions of the manganese compound. It has been found that higher mole ratios, i.e. above 3:1, do not give sufficient added inhibition to warrant the increased cost of using such larger amounts of the inhibitor.

I claim:

1. A composition adapted for use as a stable antiknock additive for spark ignition internal combustion engine fuels consisting essentially of methyl cyclopentadienyl

30 manganese tricarbonyl and a hydrocarbon oil soluble beta diketone characterized by having the structural formula



35 wherein R and R' are hydrocarbon radicals selected from the group consisting of alkyl, aryl, alkaryl and aralkyl radicals containing from 1 to 20 carbon atoms, the beta-diketone being present in an amount ranging from 1 mole to 3 moles per mole of the methyl cyclopentadienyl manganese tricarbonyl.

40 2. A composition adapted for use as a stable antiknock additive for spark ignition internal combustion engine fuels consisting essentially of methyl cyclopentadienyl manganese tricarbonyl antiknock agent and isovaleryl acetone, the isovaleryl acetone being present in an amount ranging from 1 mole to 3 moles per mole of the methyl cyclopentadienyl manganese tricarbonyl antiknock agent.

45 3. A composition adapted for use as a stable anti-knock additive for spark ignition internal combustion engine fuels consisting essentially of a lead alkyl antiknock agent, methyl cyclopentadienyl manganese tricarbonyl antiknock agent and a hydrocarbon oil soluble beta-diketone characterized by having the structural formula



50 wherein R and R' are hydrocarbon radicals selected from the group consisting of alkyl, aryl, alkaryl and aralkyl radicals containing from 1 to 20 carbon atoms, the methyl

55 cyclopentadienyl manganese tricarbonyl being present in an amount such that the weight ratio of the manganese

to the lead of the lead alkyl ranges from 1:63 to 1:1 and the beta diketone being present in an amount ranging from 1 mole to 3 moles per mole of the methyl cyclopentadienyl manganese tricarbonyl.

4. The composition of claim 3, wherein the weight ratio of the manganese of the methyl cyclopentadienyl manganese tricarbonyl to the lead of the lead alkyl ranges from 1:24 to 1:2 and the beta-diketone ranges from 1 mole to 3 moles per mole of the methyl cyclopentadienyl manganese tricarbonyl.

5. A composition adapted for use as a stable antiknock additive for spark ignition internal combustion engine fuels consisting essentially of tetraethyl lead antiknock agent, methyl cyclopentadienyl manganese tricarbonyl antiknock agent and a hydrocarbon oil soluble beta-diketone characterized by having the structural formula



wherein R and R' are hydrocarbon radicals selected from the group consisting of alkyl, aryl, alkaryl and aralkyl radicals containing from 1 to 20 carbon atoms, the methyl cyclopentadienyl manganese tricarbonyl being present in an amount such that the weight ratio of the manganese to the lead of the tetraethyl lead ranges from 1:63 to 1:1 and the beta diketone being present in an amount ranging from 1 mole to 3 moles per mole of the methyl cyclopentadienyl manganese tricarbonyl.

6. The composition of claim 5 wherein the weight ratio of the manganese of the methyl cyclopentadienyl manganese tricarbonyl to the lead of the tetraethyl lead ranges from 1:24 to 1:2 and the beta diketone ranges from 1 mole to 3 moles per mole of the methyl cyclopentadienyl manganese tricarbonyl.

7. A composition adapted for use as a stable antiknock additive for spark ignition internal combustion engine fuels consisting essentially of tetraethyl lead antiknock agent, methyl cyclopentadienyl manganese tricarbonyl antiknock agent and isovaleryl acetone, the methyl cyclopentadienyl manganese tricarbonyl being present in an amount such that the weight ratio of the manganese to the lead of the tetraethyl lead ranges from 1:63 to 1:1 and the isovaleryl acetone being present in an amount ranging from 1 mole to 3 moles per mole of the methyl cyclopentadienyl manganese tricarbonyl.

8. The composition of claim 7 wherein the weight ratio of the manganese of the methyl cyclopentadienyl manganese tricarbonyl to the lead of the tetraethyl lead ranges from 1:24 to 1:2 and the isovaleryl acetone ranges from 1 mole to 3 moles per mole of the methyl cyclopentadienyl manganese tricarbonyl.

9. A fuel composition for use in spark ignition internal combustion engines consisting essentially of a petroleum fraction boiling in the gasoline hydrocarbon range, which gasoline fuel is stable toward gum formation and a stable antiknock composition consisting essentially of methyl cyclopentadienyl manganese tricarbonyl and a hydrocarbon oil soluble beta-diketone characterized by having the structural formula



wherein R and R' are hydrocarbon radicals selected from the group consisting of alkyl, aryl, alkaryl and aralkyl radicals containing from 1 to 20 carbon atoms, the manganese of the methyl cyclopentadienyl manganese tricarbonyl ranging in an amount from 0.1 gram to 6.3 grams per gallon of gasoline and the beta-diketone being present in an amount ranging from 1 mole to 3 moles per mole of the methyl cyclopentadienyl manganese tricarbonyl.

10. A fuel composition for use in spark ignition internal combustion engines consisting essentially of a petroleum fraction boiling in the gasoline hydrocarbon range, which gasoline fuel is stable toward gum-formation and a stable antiknock composition consisting essentially of methyl cyclopentadienyl manganese tricarbonyl and isovaleryl acetone, the manganese of the methyl cyclopentadienyl manganese tricarbonyl ranging in an amount from 0.1 gram to 6.3 grams per gallon of gasoline and the isovaleryl acetone being present in an amount ranging from 1 mole to 3 moles per mole of the methyl cyclopentadienyl manganese tricarbonyl.

11. A fuel composition for use in spark ignition internal combustion engines consisting essentially of a petroleum fraction boiling in the gasoline hydrocarbon range, which gasoline fuel is stable toward gum-formation and a stable antiknock composition consisting essentially of a lead alkyl antiknock agent, methyl cyclopentadienyl manganese tricarbonyl antiknock agent, and a hydrocarbon oil soluble beta-diketone characterized by having the structural formula



25 wherein R and R' are hydrocarbon radicals selected from the group consisting of alkyl, aryl, alkaryl and aralkyl radicals containing from 1 to 20 carbon atoms, the lead of the lead alkyl antiknock agent ranging from 0.1 gram to 6.3 grams per gallon of gasoline, the manganese of the methyl cyclopentadienyl manganese tricarbonyl ranging in an amount from 0.1 gram to 6.3 grams per gallon of gasoline and the beta-diketone being present in an amount ranging from 1 mole to 3 moles per mole of the methyl cyclopentadienyl manganese tricarbonyl.

30 35 12. A fuel composition for use in spark ignition internal combustion engines consisting essentially of a petroleum fraction boiling in the gasoline hydrocarbon range, which gasoline fuel is stable toward gum-formation and a stable antiknock composition consisting essentially of a lead alkyl antiknock agent, methyl cyclopentadienyl manganese tricarbonyl antiknock agent, and isovaleryl acetone, the lead of the lead alkyl antiknock agent ranging from 0.1 gram to 6.3 grams per gallon of gasoline, the manganese of the methyl cyclopentadienyl manganese tricarbonyl ranging in an amount from 0.1 gram to 6.3 grams per gallon of gasoline and the isovaleryl acetone being present in an amount ranging from 1 mole to 3 moles per mole of the methyl cyclopentadienyl manganese tricarbonyl.

#### References Cited by the Examiner

##### UNITED STATES PATENTS

|           |         |                  |       |       |
|-----------|---------|------------------|-------|-------|
| 2,176,747 | 10/1939 | Schneider et al. | ----- | 44-69 |
| 2,197,477 | 4/1940  | Lyons et al.     | ----- | 44-77 |
| 2,316,012 | 4/1943  | Miller           | ----- | 44-77 |
| 2,818,417 | 12/1957 | Brown et al.     | ----- | 44-68 |
| 2,953,587 | 9/1960  | Clinton et al.   | ----- | 44-68 |
| 3,004,070 | 10/1961 | Hartle           | ----- | 44-78 |

##### FOREIGN PATENTS

|         |         |                |
|---------|---------|----------------|
| 590,053 | 10/1960 | Belgium.       |
| 575,637 | 2/1946  | Great Britain. |
| 851,587 | 10/1960 | Great Britain. |

##### OTHER REFERENCES

65 "On Hydrogen Bonds Intimately Related With Electron Systems," by Masamichi Tsuboi, Bulletin of Chemical Society of Japan, vol. 25, 1952, pp. 385-392.

70 DANIEL E. WYMAN, Primary Examiner.

JULIUS GREENWALD, Examiner.

Y. M. HARRIS, Assistant Examiner.